

## UNITED STATES PATENT OFFICE

ALBERT W. MORRIS, OF SPRINGFIELD, MASSACHUSETTS, ASSIGNOR TO MOORE DROP FORGING COMPANY, OF SPRINGFIELD, MASSACHUSETTS, A CORPORATION OF MASSACHUSETTS

## CAST FERROUS NITRIDED ARTICLE

No Drawing. Application filed November 21, 1931. Serial No. 576,820.

This invention relates to a cast ferrous article having a superior wearing surface produced by the so-called nitriding process.

Difficulty has been found in producing a cast iron article having a nitrided surface. By cast iron I mean an alloy of iron containing from 1.7% to 3.75% of carbon.

The alloy that I particularly am aiming to improve is an iron alloy containing 2.40% to 2.75% of carbon.

I have discovered from experiment and research that this particular alloy can be readily prepared for the nitriding process by simply adding about 1% to 2% of zirconium to the molten alloy, it being unnecessary to add any other element except the zirconium.

The zirconium is added to the molten iron alloy preferably in the form of zirconium silicate in an amount proper to add 1% to 2% of pure zirconium to the mixture.

After the mixture is formed the same is poured into a mold to form the article. After this casting has set or cooled, the same is submitted to a nitriding process whereby it is subjected to free nitrogen which will combine with and nitrate or harden the surface of the article.

By using the particular percent of zirconium specified and practically no other element, I have found that cast iron as above defined can be cheaply and efficiently nitrided.

The article thus produced may be malleableized or heat treated in addition to being nitrided, and machined or ground to exact size or shape.

The cast article thus made has the following advantages.

1. It will die cast and the alloying elements will not have sufficient affinity for oxygen or any other gas to form any compound that causes non-metallic inclusion. This is not true of other alloys used for this purpose such as those containing aluminum.

2. It can be straightened while hot, something which is desirable as most long castings leave the mold warped or twisted.

3. It can be heat treated in a reasonable time, say two hours, and at a reasonable cost. 50 This is not true of ordinary malleable iron.

4. It will nitride to a hardness of at least 600 Vickers brinell. This is only true of very few alloys.

5. During nitrogenation the casting will remain stable; that is, the nitriding temperature will not warp it.

6. While the casting will grow while it is being nitrided it will grow uniformly so that the growth can be calculated.

7. The casting will finish with a steel like 60 surface; that is, with no free carbon showing. Any free carbon is present only as temper carbon.

Having thus described my invention, what I claim as new and desire to secure by Letters Patent of the United States, is:—

1. As a new article of manufacture, a cast ferrous article, substantially free of aluminum, and containing from 1.7 percent to 3.75 percent of carbon and one to two percent of zirconium and having its surface hardened by nitriding.

2. As a new article of manufacture, a cast ferrous article containing from 1.7 percent to 3.75 percent of carbon and one to two percent of zirconium and substantially no other element, and having its surface hardened by the nitriding process.

3. As a new article of manufacture, a cast iron article, substantially free of aluminum and containing one to two percent of zirconium and having its surface hardened by nitriding.

In testimony whereof I have hereunto affixed my signature.

ALBERT W. MORRIS.

90

95

100